



US008124547B2

(12) **United States Patent**  
**Rockenfeller et al.**

(10) **Patent No.:** **US 8,124,547 B2**  
(45) **Date of Patent:** **\*Feb. 28, 2012**

(54) **PENETRATION RESISTANT ARTICLES**

(75) Inventors: **Uwe Rockenfeller**, Boulder City, NV (US); **Kaveh Khalili**, Boulder City, NV (US)

(73) Assignee: **Rocky Research**, Boulder City, NV (US)

(\*) Notice: Subject to any disclaimer, the term of this patent is extended or adjusted under 35 U.S.C. 154(b) by 26 days.

This patent is subject to a terminal disclaimer.

(21) Appl. No.: **12/688,649**

(22) Filed: **Jan. 15, 2010**

(65) **Prior Publication Data**

US 2010/0119747 A1 May 13, 2010

**Related U.S. Application Data**

(63) Continuation-in-part of application No. 11/029,685, filed on Jan. 4, 2005, now Pat. No. 7,648,757.

(51) **Int. Cl.**

*D04H 13/00* (2006.01)  
*F41H 5/00* (2006.01)  
*B32B 5/02* (2006.01)  
*B32B 27/12* (2006.01)

(52) **U.S. Cl.** ..... **442/86**; 428/174; 428/213; 428/222; 428/300.1; 428/36.4; 442/59; 442/286; 2/2.5

(58) **Field of Classification Search** ..... None  
See application file for complete search history.

(56) **References Cited**

**U.S. PATENT DOCUMENTS**

|                 |        |                                  |
|-----------------|--------|----------------------------------|
| 4,311,630 A     | 1/1982 | Humphrey et al.                  |
| 4,351,878 A     | 9/1982 | Harper-Tervet et al.             |
| 6,224,842 B1    | 5/2001 | Rockenfeller et al.              |
| 6,736,194 B2    | 5/2004 | Rockenfeller et al.              |
| 7,722,952 B2 *  | 5/2010 | Rockenfeller et al. .... 428/380 |
| 2006/0147710 A1 | 7/2006 | Rockenfeller et al.              |

**OTHER PUBLICATIONS**

Restriction Requirement dated Mar. 27, 2008 in U.S. Appl. No. 11/029,686.

Office Action dated Jun. 27, 2008 in U.S. Appl. No. 11/029,686.  
Department of Defense Handbook; Composite Materials Handbook, vol. 1, Ch. 3, pp. 2-3.

Final Office Action dated Dec. 12, 2008 in U.S. Appl. No. 11/029,686.

Advisory Action dated Feb. 25, 2009 in U.S. Appl. No. 11/029,686.  
Office Action dated May 15, 2009 in U.S. Appl. No. 11/029,686.

\* cited by examiner

*Primary Examiner* — Jennifer Chriss

*Assistant Examiner* — Camie Thompson

(74) *Attorney, Agent, or Firm* — Knobbe, Martens, Olson & Bear LLP

(57) **ABSTRACT**

A penetration resistant composite comprises a substrate material comprising woven, layered or intertwined polarized strands of glass, polyamide, polyphenylene sulfide, carbon or graphite fibers, a salt, oxide, hydroxide or hydride of a metal selected from the group consisting of alkali metal, alkaline earth metal, transition metal, zinc, cadmium, tin, aluminum, double metal salts and/or mixtures of two or more thereof or a metal hydride polar bonded on the surface of said fibers and/or strands of fibers at a concentration of at least about 0.3 grams/cc of open substrate material volume, and a substantially water impermeable coating thereon.

**34 Claims, No Drawings**

## PENETRATION RESISTANT ARTICLES

## CROSS-REFERENCE TO RELATED APPLICATIONS

This application is a continuation-in-part of U.S. patent application Ser. No. 11/029,685 filed Jan. 4, 2005 and now U.S. Pat. No. 7,648,757 issued on Jan. 19, 2010.

## BACKGROUND OF THE INVENTION

Penetration resistant materials presently available for protecting unarmored vehicles and personnel from small arms projectile penetration or penetration from flying shrapnel and the like are relatively expensive. The compositions described herein are relatively inexpensive and cost-effective to manufacture. The materials comprise a composite which may be produced in almost any shape, size and thickness, and are fully recyclable.

## SUMMARY OF THE INVENTION

The penetration resistant composites described herein comprise a substrate material comprised of woven, layered or intertwined polarized strands of glass, polyamide, polyphenylene sulfide, carbon or graphite fibers on which a selected metal, salt, oxide, hydroxide or metal hydride is polar bonded on the surface of the fibers and/or strands at concentrations sufficient to form bridges of the salt, oxide, hydroxide or hydrides between adjacent substrate strands and/or substrate fibers. Single or multiple layers of the salt or hydride bonded fibers are coated with a substantially water impermeable coating material. Panels or other shaped penetration resistant products may be produced using composite layers.

## DETAILED DESCRIPTION

The penetration resistant composite products described herein are fabricated from a substrate material comprising woven or intertwined polarized strands or layered strands of the substrate. Such woven or intertwined substrate material incorporate or utilize elongated or continuous fibers such as fabrics or cloth or unwoven intertwined fiber materials such as yarn, rope or the like where the fibers or strands of fibers have been twisted or formed in a coherent form such as yarn or weaves of strands. Various or different weaving patterns may be used, preferably three-dimensional weaves which yield multi-directional strength characteristics as compared to two-dimensional weaves having anisotropic strength characteristics. Moreover, the substrate utilizes elongated and/or continuous fibers or filaments as opposed to chopped or loose fibers or strands in which there is no interlocking or structural pattern to the fibrous substrate. Suitable materials also include needle woven layers of substrate fiber strands. Alternatively, layers of elongated, substantially continuous fiber strands which have not been woven in a three-dimensional weave may be used. Successive layers of the fibers are preferably positioned along different axes so as to give the substrate strength in multiple directions. Moreover, such layers of non-woven fibers can be positioned between layers of woven fibers.

The substrate material of which the fiber strands are made include glass, polyamide, polyphenylene sulfide, carbon or graphite fibers. Glass fibers are a preferred fiber material, woven glass fibers being relatively inexpensive and woven glass fiber fabric easy to handle and process in preparing the composites. The glass fibers may be E-glass and/or S-glass,

the latter having a higher tensile strength. Glass fiber fabrics are also available in many different weaving patterns which also makes the glass fiber material a good candidate for the composites. Carbon and/or graphite fiber strands may also be used. Polyamide materials or nylon polymer fiber strands are also useful, having good mechanical properties. Aromatic polyamide resins (aramid resin fiber strands, commercially available as Kevlar® and Nomex®) are also useful. Yet another useful fiber strand material is made of polyphenylene sulfide, commercially available as Ryton®. Combinations of two or more of the aforesaid materials may be used in making up the substrate, with specific layered material selected to take advantage of the unique properties of each of them. The substrate material, preferably has an open volume of at least about 30%, and more preferably 50% or more, up to about 90%.

The surface of the fibers and fiber strands of the aforesaid substrate material may be polarized. Polarized fibers are commonly present on commercially available fabrics, weaves or other aforesaid forms of the substrate. If not, the substrate may be treated to polarize the fiber and strand surfaces. The surface polarization requirements of the fiber, whether provided on the substrate by a manufacturer, or whether the fibers are treated for polarization, should be sufficient to achieve a loading density of the salt on the fiber of at least about 0.3 grams per cc of open substrate volume in one embodiment, whereby the bonded metal salt bridges adjacent fiber and/or adjacent strands of the substrate. Polarity of the substrate material may be readily determined by immersing or otherwise treating the substrate with a solution of the salt, drying the material and determining the weight of the salt polar bonded to the substrate. Alternatively, polar bonding may be determined by optically examining a sample of the dried substrate material and observing the extent of salt bridging of adjacent fiber and/or strand surfaces. Even prior to such salt bonding determination, the substrate may be examined to see if oil or lubricant is present on the surface. Oil coated material may in some circumstances substantially negatively affect the ability of the substrate fiber surfaces to form an ionic, polar bond with a metal salt or hydride. If surface oil is present, the substrate may be readily treated, for example, by heating the material to sufficient temperatures to burn off or evaporate the undesirable lubricant. Oil or lubricant may also be removed by treating the substrate with a solvent, and thereafter suitably drying the material to remove the solvent and dissolved lubricant. Substrates may also be treated with polarizing liquids such as water, alcohol, inorganic acids, e.g., sulfuric acid.

The substrate may be electrostatically charged by exposing the material to an electrical discharge or "corona" to improve surface polarity. Such treatment causes oxygen molecules within the discharge area to bond to the ends of molecules in the substrate material resulting in a chemically activated polar bonding surface. Again, the substrate material should be substantially free of oil prior to the electrostatic treatment in some embodiments.

In one embodiment, a metal salt, metal oxide, hydroxide or metal hydride, is bonded to the surface of the polarized substrate material by impregnating, soaking, spraying, flowing, immersing or otherwise effectively exposing the substrate surface to the metal salt, oxide, hydroxide or hydride. A preferred method of bonding the salt to the substrate is by impregnating, soaking, or spraying the material with a liquid solution, slurry or suspension or mixture containing the metal salt, oxide, hydroxide or hydride followed by removing the solvent or carrier by drying, heating and/or by applying a vacuum. The substrate may also be impregnated by pumping a salt suspension, slurry or solution or liquid-salt mixture into

and through the material. Where the liquid carrier is a solvent for the salt, it may be preferred to use a saturated salt solution for impregnating the substrate. However, for some cases, lower concentrations of salt may be used, for example, where necessitated or dictated to meet permissible loading densities. Where solubility of the salt in the liquid carrier is not practical or possible, substantially homogeneous dispersions may be used. Where an electrostatically charged substrate is used, the salt may be bonded by blowing or dusting the material with dry salt or hydride particle.

As previously described, in some embodiments, it may be necessary to bond a sufficient amount of metal salt, oxide, hydroxide or hydride on the substrate to achieve substantial bridging of the salt, oxide, hydroxide or hydride crystal structure between adjacent fibers and/or strands. A sufficient amount of metal salt, oxide, hydroxide or hydride is provided by at least about 0.3 grams per cc of open substrate volume, preferably at least about 0.4 grams per cc, and most preferably at least about 0.5 grams per cc of open substrate volume, which is between about 30% and about 95% of the untreated substrate volume, and preferably between about 50% and about 90% of the untreated substrate volume. Following the aforesaid treatment, the material is dried in equipment and under conditions to form a flat layer, or other desired size and shape using a mold or form. A dried substrate will readily hold its shape. In one embodiment, the substrate is dried to substantially eliminate the solvent, carrier fluid or other liquid, although small amounts of fluid, for example, up to 1-2% of solvent, can be tolerated without detriment to the strength of the material. Drying and handling techniques for such solvent removal will be understood by those skilled in the art.

The metal salts, oxides or hydroxides bonded to the substrate are alkali metal, alkaline earth metal, transition metal, zinc, cadmium, tin, aluminum, double metal salts of the aforesaid metals, and/or mixtures of two or more of the metal salts. The salts of the aforesaid metals may be halide, nitrite, nitrate, oxalate, perchlorate, sulfate or sulfite. The preferred salts may include halides, and preferred metals may include strontium, magnesium, manganese, iron, cobalt, calcium, barium and lithium. The aforesaid preferred metal salts provide molecular weight/electrovalent (ionic) bond ratios of between about 40 and about 250. Hydrides of the aforesaid metals may also be useful, examples of which are disclosed in U.S. Pat. Nos. 4,523,635 and 4,623,018, incorporated herein by reference in their entirety.

Following the drying step or where the salts are bonded to dry, electrostatically charged substrate, if not previously sized, the material is cut to form layers of a desired size and/or shape, and each layer of metal salt or hydride bonded substrate material or multiple layers thereof are sealed by coating with a substantially water-impermeable composition. The coating step should be carried out under conditions or within a time so as to substantially seal the composite thereby preventing the metal salt or hydride from becoming hydrated via moisture, steam, ambient air, or the like, which may cause deterioration of strength of the material. The timing and conditions by which the coating is carried out will depend somewhat on the specific salt bonded on the substrate. For example, calcium halides, and particularly calcium chloride and calcium bromide will rapidly absorb water when exposed to atmospheric conditions causing liquefaction of the salt and/or loss of the salt bond and structural integrity of the product. Substantially water-impermeable coating compositions include epoxy resin, phenolic resin, neoprene, vinyl polymers such as PBC, PBC vinyl acetate or vinyl butyral copolymers, fluoroplastics such as polychlorotrifluoroethylene, polytetrafluoroethylene, FEP fluoroplastics, polyvi-

nylidene fluoride, chlorinated rubber, and metal films including aluminum and zinc coatings. The aforesaid list is by way of example, and is not intended to be exhaustive. Again, the coating may be applied to individual layers of substrate, and/or to a plurality of layers or to the outer, exposed surfaces of a plurality or stack of substrate layers.

Panels or other forms and geometries such as concave, convex or round shapes of the aforesaid coated substrate composites such as laminates are formed to the desired thickness, depending on the intended ballistic protection desired, in combination with the aforesaid composites to further achieve desired or necessary performance characteristics. For example, useful panels or laminates of such salt bonded woven substrates may comprise 10-50 layers per inch thickness. Such panels or laminates may be installed in doors, sides, bottoms or tops of a vehicle to provide armor and projectile protection. The panels may also be assembled in the form of cases, cylinders, boxes or containers for protection of many kinds of ordnance or other valuable and/or fragile material such as ammunition, fuel and missiles as well as personnel. Laminates may include layers of steel or other ballistic resistant material such as carbon fiber composites, aramid composites or metal alloys.

The aforesaid composites may be readily molded into articles having contoured and cylindrical shapes, specific examples of which include helmets, helmet panels or components, vests, vest panels as well as vehicle protection panels, vehicle body components, rocket or missile housings and rocket or missile containment units, including NLOS (non line of sight) systems. Such housings and containment units would encase and protect a rocket or missile and are used to store and/or fire missiles or rockets and could be constructed using the composites described herein to protect their contents from external objects such as bullets or bomb fragments. Vest panels of various sizes and shapes may be formed for being inserted into pockets located on or in the lining of existing or traditional military vests. The combined use of such panels with more traditional bulletproof vests may result in a lighter, more flexible, and more readily adaptable vest that accommodates the variety of sizes for different individuals. Similarly, one embodiment is a helmet panel that has been contoured to fit inside as a liner for a traditional helmet. In another embodiment, the protective composite panel is secured on the outside of the helmet with flexible and/or resilient helmet covers, netting, etc. In a different embodiment, the helmet may include one or more contoured or shaped composites as described herein to protect the wearer from bullets or bomb fragments.

For penetration resistant vehicular armor, many different sized and shaped protection panels may be formed of the composite including floor, door, side and top panels as well as vehicle body components contoured in the shape of fenders, gas tank, engine and wheel protectors, hoods, and the like. As used herein, "vehicle" includes a variety of machines, including automobiles, tanks, trucks, helicopters, aircraft and the like. Thus, the penetration resistant vehicle armor may be used to protect the occupants or vital portions of any type of vehicle.

The aforesaid composite articles may also be combined with other ballistic and penetration resistant panels of various shapes and sizes. For example, the aforesaid composites may be paired with one or more layers or panels of materials such as steel, aramid resins, carbon fiber composites, boron carbide, or other such penetration resistant materials known to those skilled in the art including the use of two or more of the aforesaid materials, depending on the armor requirements of the penetration resistant articles required.

By way of example, a woven glass fiber substrate bonded with strontium chloride was formed according to the previously described procedure at a concentration of 0.5 grams salt per cc of open substrate space. Layers of the substrate were coated with epoxy resin and formed in a panel 12.5 in. x 12.5 in. x 0.5 in. thick. The panel weighed 4.71 pounds, having material density of 0.06 pounds per cubic inch, comparing to 22% of the density of carbon steel. Bullets fired from a military-issued Beretta gun firing 9 mm 124-grain FMG bullets (9 g PMC stock number, full metal jacket), at 20 yards did not fully penetrate the panel.

What is claimed is:

1. A composite panel comprising a composite of a substrate material comprising:

one or more layers of polarized strands of fibers;  
a salt, oxide, hydroxide or hydride of a metal polar bonded on the surface of said fibers at a concentration of at least about 0.3 grams/cc of open substrate material volume; and  
a substantially water impermeable coating composition on the one or more layers or an exterior surface of said composite.

2. A composite panel of claim 1, wherein the panel comprises a panel of body armor configured to protect a person.

3. A composite panel of claim 1, wherein the panel comprises a panel of vehicle armor configured to protect a vehicle.

4. A composite panel of claim 1, wherein the fibers comprise woven, layered or intertwined polarized strands of glass, polyamide, polyphenylene sulfide, carbon or graphite fibers.

5. A composite panel of claim 1, wherein the substantially water impermeable coating composition is on an exterior surface of said composite.

6. A composite panel of claim 1, wherein the panel comprises a vehicle body component.

7. A composite panel of claim 1, wherein the panel has a concave, convex or round shape.

8. A composite panel of claim 1, wherein the panel comprises 10 to 50 layers per inch of panel thickness.

9. A composite panel of claim 1, wherein the panel is assembled into the form of a protective box or container.

10. A composite panel of claim 1, further comprising, in addition to said layers of polarized strands of fibers, one or more layers or panels of steel, carbon fiber composite, aramid resin, boron carbide, or a combination of two or more thereof.

11. A composite panel of claim 1, comprising a shaped personnel protection panel, vehicle protection panel or vehicle body component.

12. A composite panel of claim 11, wherein said fibers comprise woven, layered or intertwined polarized strands of glass, polyamide, polyphenylene sulfide, carbon or graphite fibers.

13. A composite panel of claim 11, wherein the metal comprises one or more of an alkali metal, alkaline earth metal, transition metal, zinc, cadmium, tin, aluminum, or double metal salts.

14. A composite panel of claim 11, wherein said salt comprises a halide, nitrite, nitrate, oxalate, perchlorate, sulfate or sulfite of said metal.

15. A composite panel of claim 11 comprising a plurality of layers of woven or intertwined polarized strands of fibers.

16. A composite panel of claim 11, wherein the polarized strands comprise aromatic polyamide resin fibers.

17. A composite panel of claim 11, wherein the polarized strands comprise combinations of two or more different polarized strand materials.

18. A composite panel comprising a composite of a substrate material comprising:

one or more layers of polarized strands of fibers;  
a salt, oxide, hydroxide or hydride of a metal polar bonded on the surface of said fibers;  
a substantially water impermeable coating composition on the one or more layers or an exterior surface of said composite; and

wherein the panel comprises 10 to 50 layers of said polarized strands of fibers per inch of panel thickness.

19. A composite panel of claim 18, wherein the panel comprises a panel of body armor configured to protect a person.

20. A composite panel of claim 18, wherein the panel comprises a panel of vehicle armor configured to protect a vehicle.

21. A composite panel of claim 18 wherein the fibers are present at a concentration of at least about 0.3 grams/cc of open substrate material volume.

22. A composite panel of claim 18, wherein the fibers comprise woven, layered or intertwined polarized strands of glass, polyamide, polyphenylene sulfide, carbon or graphite fibers.

23. A composite panel of claim 18, wherein the substantially water impermeable coating composition is on an exterior surface of said composite.

24. A composite panel of claim 18, wherein the panel comprises a vehicle body component.

25. A composite panel of claim 18, wherein the panel has a concave, convex or round shape.

26. A composite panel of claim 18, wherein the panel is assembled into the form of a protective box or container.

27. A composite panel of claim 18, further comprising, in addition to said layers of polarized strands of fibers, one or more layers or panels of steel, carbon fiber composite, aramid resin, boron carbide, or a combination of two or more thereof.

28. A composite panel of claim 18, comprising a shaped personnel protection panel, vehicle protection panel or vehicle body component.

29. A composite panel of claim 28, wherein said fibers comprise woven, layered or intertwined polarized strands of glass, polyamide, polyphenylene sulfide, carbon or graphite fibers.

30. A composite panel of claim 28, wherein the metal comprises one or more of an alkali metal, alkaline earth metal, transition metal, zinc, cadmium, tin, aluminum, or double metal salts.

31. A composite panel of claim 28, wherein said salt comprises a halide, nitrite, nitrate, oxalate, perchlorate, sulfate or sulfite of said metal.

32. A composite panel of claim 28 comprising a plurality of layers of woven or intertwined polarized strands of fibers.

33. A composite panel of claim 28, wherein the polarized strands comprise aromatic polyamide resin fibers.

34. A composite panel of claim 28, wherein the polarized strands comprise combinations of two or more different polarized strand materials.